

Dec. 15, 1931.

E. F. KOHMAN

1,837,051

FOOD CONTAINER

Filed April 10, 1928



Inventor

E. F. KOHMAN

By

Semmes & Semmes

Attorney

## UNITED STATES PATENT OFFICE

EDWARD F. KOHMAN, OF WASHINGTON, DISTRICT OF COLUMBIA, ASSIGNOR TO  
NATIONAL CANNERS ASSOCIATION, OF WASHINGTON, DISTRICT OF COLUMBIA, A  
CORPORATION OF DELAWARE

## FOOD CONTAINER

Application filed April 10, 1928. Serial No. 271,417.

This invention relates to food receptacles, and more particularly to an improved container for canned foods.

One of the sources of losses in the production and distribution of canned foods is the so termed hydrogen swells.

These swells are caused by corrosion of the can and the consequent evolution of hydrogen. As is known when a metal, such as iron, dissolves in acid an equivalent amount of hydrogen is evolved. The losses arising from hydrogen swells, therefore, are of particular importance in the canning of acid foods, such as fruit products.

15 It is an object of this invention to provide a metallic container which minimizes the formation of hydrogen.

Another object of this invention is to provide a food container which comprises metals of different electro-chemical characteristics.

A further object of this invention is to provide a container in which perforations are minimized.

25 Yet another object is to provide a container which comprises metals of different physical properties.

A further object is to provide a novel can top adapted for use with a tin can.

30 With these and other equally important objects in view, the invention comprehends the provision of a can, comprising a body and ends of metals of different characteristics, and which are so related as to minimize 35 perforations and the formation of hydrogen.

The invention is illustrated diagrammatically in the single figure of the accompanying drawing. In this the numeral A represents a can body of the usual type and B indicates a covering composed of a softer metal than the metal comprising the body. Thus the covering B provides an end or top for 45 the can.

It has long been known that perforations resulting from various fruits in enameled cans occur very largely at the countersunk end of the can. It has been assumed that 50 the source of hydrogen formation is this

countersink portion, since it is at the point where the perforations occur.

As a result of extended experiments, I have found that a large part of the hydrogen and, in some instances, the majority of it may be the result of corrosion at points of the can other than the countersink. The portions 55 where the corrosion usually centers is on that section of the can body which projects into the double seam and is adjacent to the countersink on the end. The corrosion at this point is more pronounced when a rubber compound lining is used than is the case where a paper gasket is employed.

These observations clearly indicate that 60 corrosion on the body of the can is due to the injury received, or the strained condition resulting from the stresses imposed during the double seaming operation. This injury as has been stated, may be diminished 65 by interposing a member, such as a paper gasket, which provides a padding or buffer effect.

I have found that the generation of hydrogen is initiated considerably sooner, and its 70 deleterious effects made quickly manifest, if the deformation of the can body is accentuated, as evidenced by the following experiment. A certain number of tin cans of the 75 usual type were filled with red raspberries. Cans of this type of fruit, as is well known, 80 are not particularly susceptible to hydrogen formation. These cans were then sealed with stainless steel tops. These tops, as will be 85 understood, are not corroded by red raspberries or by any of the other acid food products. This metal, it will be noted, is of a 90 stiffer or harder character than the metal of the can body. After a period of three months, each of these cans had become a hydrogen swell. The significance of the factor will be 95 fully appreciated when it is considered that similar cans, with a tin plate top, generally show no hydrogen formation for a period considerably more than a year.

The cans used in this experiment were 100 opened and it was then found that the corrosion noticed in enameled tin cans of this type was greatly augmented. Upon examination of the seams, it was immediately evi-

denced that the ruffles which were formed on the edge of the end from the first operation of the double seamer, caused indentations in the contiguous section of the body of the can. 5 These indentations were plainly visible to the naked eye.

This deformation of the metal of the can body disrupted the enameled inside surface of the can, and corrosion started at, 10 and spread from, these points. It was noted that these indentations were similar although much augmented to indentations that are sometimes noticeable on ordinary commercial cans. From an inspection of a number of 15 commercial cans, at different stages of storage, it appears that the corrosion initiates at the protuberances or indentations caused by the double seaming operation and emanating from these points merges into a band of 20 corroded area encircling the entire can near the edge.

I have found that this deformation of the can and its concomitant disadvantages may be avoided by providing a can body which 25 will not deform when it is seamed in. This as shown in the drawing may be accomplished in two general ways; first, by providing a top or cover which is of a softer or more deformable material than the can body, or by making the can body itself of greater rigidity or 30 stiffness than has been done heretofore. Whether the can body and its ends are constructed of the same material but of varying thickness, or whether the can body is constructed of one metal or alloy and the deformable top of a different metal or alloy, 35 it will be appreciated that the body of the can is heavier than the ends or top, inasmuch as the former offers greater resistivity to deformation than the latter portion. It is to be understood that the word "heavier" is employed in this sense in the claims appended 40 hereto.

The advantages of this invention may be 45 secured by utilizing an aluminum or aluminum alloy top in conjunction with a can body of the usual type. As is known, aluminum material, and many other alloys, is much softer than the ferruginous base plate and, 50 hence will distort before the can body. It will immediately be perceived that by utilizing such a top any deformation incident to the seaming operation will be limited to or concentrated in the top.

55 Aluminum and aluminous alloys are particularly well adapted to the present use. In its electro-chemical effect in relation to the iron of the base plate, aluminum is comparable to tin. The electro-chemical effect of 60 tin in a tin can is to inhibit the corrosion of iron, while on the other hand the corrosion of tin is augmented as a result of being in contact with iron. The corrosion of tin, however, is exceedingly small, since the area of iron 65 which is exposed as compared to the area of

tin is quite small. As will be seen from an inspection of the following tables the corrosion test with aluminum and base plate disclose a similar relationship existing between aluminum and iron, as that which obtains 70 between tin and iron. The corrosion of iron is inhibited by virtue of its being in contact with aluminum. It is particularly to be noted that aluminum possesses an advantage over 75 tin in the fact that the corrosion of aluminum is not increased by contact with iron in the base plate. It will be seen, therefore, that an aluminum end on a tin plate body will have a beneficial electro-chemical effect. As has 80 been noted hereinbefore, the softness of aluminum and its alloys will prevent injuring of that portion of the tin plate body which enters into the double seam.

*Loss in milligrams or specimens of aluminum and of aluminum alloy 2 1/2×4 cm. in dimension both when alone and also when in electrical contact with iron and exposed to red raspberries as the corrosive medium*

| 210 hours                                                  |     |         |     | 523 hours  |     |         |     | 1195 hours |     |         |     | 90  |
|------------------------------------------------------------|-----|---------|-----|------------|-----|---------|-----|------------|-----|---------|-----|-----|
| No contact                                                 |     | Contact |     | No contact |     | Contact |     | No contact |     | Contact |     | 95  |
| Fe                                                         | Al  | Fe      | Al  | Fe         | Al  | Fe      | Al  | Fe         | Al  | Fe      | Al  | 95  |
| <b>ALUMINUM ALLOY (containing about 11 1/2% manganese)</b> |     |         |     |            |     |         |     |            |     |         |     |     |
| 2.1                                                        | 0.5 | 1.3     | 0.4 | 4.4        | 0.8 | 2.3     | 0.7 | 10.1       | 1.5 | 3.9     | 1.5 | 100 |
| <b>ALUMINUM</b>                                            |     |         |     |            |     |         |     |            |     |         |     |     |
| 1.6                                                        | 0.0 | 0.8     | 0.0 | 3.9        | 0.0 | 2.2     | 0.1 | 11.2       | 1.1 | 7.0     | 1.4 | 100 |

It will be observed from the foregoing 105 table, that by reason of being in contact with aluminum, the corrosion of iron is greatly diminished; for example, a specimen of iron base plate which was contacted with red raspberries as the corrosion medium lost 3.9 milligrams in approximately 22 days, whereas this material in contact with aluminum lost only 2.2 milligrams due to corrosion. The effect when using both aluminum and an aluminum alloy is particularly noticeable after the specimens have been in contact with the corrosion medium for a longer period. After an exposure of approximately 50 days, the corrosion of iron was diminished from 10.1 to 110 3.9, and from 11.2 to 7.0 milligrams when contacted with aluminum alloy and aluminum, respectively.

The table is given purely by way of example to typify the general relationship 115 which exists between the iron base plate and material of an aluminum-like nature. It will be appreciated that there are a number of specific metals and alloys which possess similar characteristics, in respect to their effect upon iron. All such metals and alloys are 120 130

comprehended within the spirit and scope of the present invention.

Aluminum and its alloys possess another decided advantage for the present use. To these materials enamel adheres very satisfactorily, in fact, in some cases the adherence is even better than the adherence of enamel to tin plate. This is of particular importance because of the fact that in the present practice those cans which are designed to contain colored acid foods are coated on the interior with an enamel.

It is to be noted that the advantages of the invention are secured at a reasonable cost. While it is true that aluminum sheets or aluminum alloys cost somewhat more than tin plate, the weight of tin plate is approximately  $2\frac{1}{2}$  times that of aluminum. Since these materials are bought by weight, it will be seen that the price of a given quantity of aluminum is about  $2\frac{1}{2}$  times less than that of tin plate.

As has been intimated hereinbefore, the advantages of the invention may be secured not only by providing a top which is of a softer material than the body portion, but also by making up the cans in the ordinary way but using a base plate of increased stiffness, that is to say, by constructing a can in which the base plate used in the body portion is stiffer or heavier than that used for the top. In this manner, when the can is subjected to the double seaming operation the metal of the top will be selectively deformed, and corrosion of the body at the place indicated will be prevented. It is to be observed that in lieu of making the base plate of the body of a heavy material, it may be constructed of the same quality as has been done hereinbefore and the can may be capped with a tin base plate which is of a lighter or less resistive character than the base plate used in the body.

The invention resides in the broad concept of providing a can in which the top and body portions are of different degrees of softness, so that when the pressure incident to the seaming operation is applied, the top of the can will be deformed, and the body retained substantially in its initial condition.

While I have shown and described the specific embodiments of the invention, it is to be understood that these are given merely by way of example, for, as has been indicated, the purpose may be effectuated by utilizing a number of different materials, hence, I do not intend to be limited to those described, except as such limitations are clearly imposed by the appended claims.

60 I claim:

1. A metal can for containing food products comprising a ferrous body portion, a thin acid-proof coating on the interior of the can body, rigid outside sustaining ends for the can, interfolded seams joining the

rigid outside sustaining ends to the can body, said ends being of softer metal than the body portion of the can.

2. A metal can for containing food products comprising a ferrous body portion enameled on the interior, rigid outside sustaining ends for the can, interfolded seams joining the rigid outside sustaining ends to the can body, said ends being of softer metal than the body portion of the can. 75

3. A metal can for containing food products comprising a ferrous body portion, a thin tin coating on the interior of the can body, rigid outside sustaining ends for the can, interfolded seams joining the rigid outside sustaining ends to the can body, said ends being of softer metal than the body portion of the can. 80

4. A metal can for containing food products comprising a ferrous body portion, a thin acid-proof coating on the interior of the can body, rigid outside sustaining ends for the can, interfolded seams joining the rigid outside sustaining ends to the can body, said ends being of an aluminous metal which is 85 softer than the body portion of the can.

5. A metal can for containing food products comprising a ferrous body portion enameled on the interior, rigid outside sustaining ends for the can, interfolded seams joining the rigid outside sustaining ends to the can body, said ends being of an aluminous metal which is softer than the body portion of the can. 95

In testimony whereof I affix my signature. 100  
EDWARD F. KOHMAN.

105

110

115

120

125

130